# EUROPEAN PATENT SPECIFICATION

(11) **EP 2 971 240 B1**
(45) Date of publication and mention of the grant of the patent: **21.11.2018**
(21) Application number: 13878078.8
(22) Date of filing: 30.12.2013
(51) Int. Cl.: C23C 28/00, C23C 28/04, C23C 4/134, C23C 4/11

(54) **HYBRID THERMAL BARRIER COATING AND PROCESS OF MAKING THE SAME**
HYBRIDE WÄRMEDÄMMSCHICHT UND VERFAHREN ZU DEREN HERSTELLUNG
REVÊTEMENT DE BARRIÈRE THERMIQUE HYBRIDE ET SON PROCÉDÉ DE FABRICATION

(30) Priority: 14.03.2013 US 201361781656 P
(43) Date of publication of application: 20.01.2016
(73) Proprietor: United Technologies Corporation, Farmington, CT 06032 (US)
(72) Inventor: HAZEL, Brian T, Avon, Connecticut 06001 (US); LITTON, David A., West Hartford, Connecticut 06107 (US); MALONEY, Michael J., Marlborough, Connecticut 06447 (US)
(74) Representative: Dehns
(86) International application number: PCT/US2013/078186
(87) International publication number: WO 2014/143363

(56) References cited:
- EP-A1- 2 336 381
- EP-A1- 2 341 166
- EP-A1- 2 450 465
- WO-A2-2014/007901
- JP-A- 2001 348 655
- JP-A- 2009 108 856
- JP-A- 2010 255 121
- KR-A- 20120 088 874
- US-A1- 2011 151 219
- US-A1- 2011 244 216

## Description

### BACKGROUND

The present disclosure relates to a thermal barrier coating for use on a turbine engine component and to a process of making the thermal barrier coating.

A thermal barrier coating (TBC) is created to meet one or more performance requirements including, but not liited to, spallation life, calcia-magnesia-alumina-silicate (CMAS) resistance, foreign object damage (FOD) resistance, erosion, and low conductivity. A turbine barrier coating is applied to a turbine engine component, such as a turbine blade/vane, to help the component withstand the relatively high temperatures of its operational environment.

TBCs are often formed using a singular coating process such as an electron beam physical vapor deposition (EB-PVD) process. For example, a TBC may be formed from two separate EB-PVD layers formed from two different materials, such as 7 wt% yttria stabilized zirconia and gadolinia stabilized zirconia in order to improve the thermal conductivity properties of the coating. The strain-tolerant columnar structure of an EB-PVD coating helps to increase the TBC spallation life. A more porous TBC however may minimize the TBC thermal conductivity and possibly the thermal radiation through the coating.

In one TBC, there is a porous outer layer over a more dense inner layer made by an EB-PVD process. In some TBCs, the two layers have different porosity levels. Such a structure can be formed by changing the coating temperature. More power equals more density but also more temperature. It is also known to form a dense vertically cracked microstructure for the TBC where the deposition is conducted at a two inch stand-off for the dense layer and a six inch stand-off for the porous layer.
EP 2 341 166 discloses a TBC on a substrate, the TBC comprising a bond coat, a ceramic coating, and a ceramic layer.

US 2011/244216 A1 discloses a combination of SPS and APS methods for deposition of multilayer thermal barrier coatings on turbine components. The applied materials comprise partially or fully YSZ as well as pyrochlores.

EP 2 336 381 A1 discloses a thermal barrier coating deposited by APS, consisting of a first 7YSZ layer and a second gadolinia stabilized zirconia layer with a porosity of 5-20 vol.%.

EP 2 450 465 A1 discloses a multilayer ceramic TBC deposited by APS, comprising an inner YSZ layer of low porosity, an intermediate YSZ layer with higher porosity than the inner layer and an outer porous layer of gadolinium zirconate.

### SUMMARY

In accordance with the present disclosure, there is provided a coating according to claim 1 and a process according to claim 3.

In another and alternative embodiment, the second layer has a porosity in the range of from 10 to 40%.

In another and alternative embodiment, the first layer forming step comprises suspending a powder feedstock in a liquid suspension and injecting the powder feedstock and the suspension into a plasma jet under conditions where the first layer is formed with the strain-tolerant columnar microstructure.

In another and alternative embodiment, the second layer forming step comprises changing spray parameters so as to form the porous and radiation thermally resistant second layer.

In another and alternative embodiment, the second layer forming step comprises forming the second layer so as to have a porosity of from 10 to 40%.

In another and alternative embodiment, the first and second layer forming steps comprise using a powdered feedstock having a particle size in the range of from 10nm to 10 micrometers

In another and alternative embodiment, the first and second layer forming steps comprises using a powdered feedstock having a particle size in the range of from 10nm to 2.0 micrometers.

Other details of the hybrid thermal barrier coating and the process of making same are set forth in the following detailed description and the accompanying drawings wherein like reference numerals depict like elements.

### BRIEF DESCRIPTION OF THE DRAWINGS

FIG. 1 illustrates a turbine engine component having a thermal barrier coating in accordance with the present disclosure deposited thereon; and
FIG. 2 illustrates a system for forming the coating on the turbine engine component.

### DETAILED DESCRIPTION

Referring now to FIG. 1, there is shown a turbine engine component 10. The turbine engine component may be any component which requires a thermal barrier coating such as a blade/vane. The turbine engine component 10 may have a substrate 12 formed from any suitable material known in the art including, but not limited to, a nickel based alloy, a cobalt based alloy, a titanium based alloy, a ceramic material, and an organo-matrix composite material.

A thermal barrier coating 14 is deposited on the substrate 12. The thermal barrier coating 14 has a first layer 16 which interfaces with the surface 18 of the substrate 12 and an outer second layer 20. The first layer 16 is formed so as to have a strain-tolerant columnar microstructure at the interface with the surface 18 of the substrate. The second layer 20 is formed to have a porous thermal conduction and radiant heat transfer resistant microstructure at an outer surface 22 of the thermal barrier coating.

The first layer 16 and the second layer 20 is formed from a material having the same composition. Each of the layers 16 and 20 is formed from a 7 wt% yttria stabilized zirconia (7YSZ).

Each of the layers 16 and 20 is formed using suspension plasma spray (SPS) technique such as that shown in FIG. 2. In this technique, a powdered feedstock is suspended in a liquid suspension 30. For example, the powdered feedstock may be 7YSZ which may be suspended in ethanol, water, or other alcohols such as methanol. The powdered feedstock may have a particle size in the range of from 10 nm to 10 micrometers mean size diameter. In another non-limiting embodiment, the particles size may be in the range of from 10 nm to 2.0 micrometers. The powdered feedstock in the suspension is injected into a plasma jet 32 created by a plasma torch 34 and thus deposited onto the substrate 12. The spray conditions are such that the first layer 16 is formed to have the desired strain tolerant columnar microstructure. The deposition technique may have a short stand off (similar to that used in dense vertically cracked coatings) and high power/enthalpy plasma conditions. After the first layer 16 has been formed, the spray conditions may be changed so as to form the second layer 20 with the porous thermal conduction and radiant heat transfer resistant microstructure. To add porosity, (1) the angle of the spray nozzle could be changed from normal relative to the surface on which the layer 20 is being deposited; (2) the stand off may be increased; and/or (3) the plasma power/enthalpy may be reduced. More porosity in the second layer 20 than in the first layer 16 creates a reduction in thermal conductivity. The second layer 20 may have a reduction of at least 10% in thermal conductivity. This may come purely from a porosity increase or a change in the structure from columnar to more splat like. An increase in porosity increases the erosion rate. A useful limit may be 10 to 40% porosity in the second layer 20.

The columnar structure SPS gives a thermal cyclic spallation resistance similar to EB-PVD (much higher than APS and higher than dense vertically cracked). Erosion is a function of porosity content and can be greater or less than EB-PVD (generally higher than APS and more like dense vertically cracked). Thermal conductivity, as discussed above, follows the porosity content.

The spray conditions are discreetly or incrementally changed throughout the spray run. The spray conditions are changed so that a continuously graded microstructure is formed where there is the strain-tolerant columnar microstructure at the interface with the substrate 12 for thermal barrier coating spallation resistance and a porous thermal conduction and radiation thermally resistant layer at the outer surface 22.

One of the advantages of the process described herein is that the thermal barrier coating can be formed using a single piece of equipment and in a single coating.

Another advantage is that one can easily change the composition of the second layer 20 so that it is different than the composition of the first layer 16. This can easily be done by changing the composition of the feedstock being injected into the plasma jet.

There has been described herein a hybrid thermal barrier coating and a process for making same.

## Claims

1. A thermal barrier coating (14) applied to a turbine engine component (10) having a substrate (2), said coating comprising:
a first layer (16) which has a strain tolerant, columnar microstructure at an interface with the substrate for spallation resistance; and
a second layer (20) which is porous, conduction and radiation thermally resistant at an outer surface of the thermal barrier coating;
wherein there is a continuously graded microstructure from the interface to the outer surface;
wherein said first and second layers are formed from the same material;
wherein each of said first and second layers is formed from 7wt% yttria stabilized zirconia; and
wherein said first layer has a first thermal conductivity and said second layer has a second thermal conductivity which is at least 10% lower than the first thermal conductivity.

2. The thermal barrier coating of claim 1, wherein said second layer has a porosity in the range of from 10 to 40%.

3. A process for applying a thermal barrier coating (14) to a turbine engine component (10) comprising:
forming a first layer (16) which has a strain tolerant columnar microstructure at an interface of the first layer and a substrate using a suspension plasma spray technique;
forming a second layer (20) which is porous and radiation thermally resistant at an outer surface of the thermal barrier coating using said suspension plasma spray technique;
forming a continuously graded microstructure from said interface to said outer surface
wherein said first and second layer forming steps comprises forming said layers from the same material;
wherein each of said first and second layers is formed from 7wt% yttria stabilized zirconia; and
wherein said second layer forming step comprises forming said second layer with more porosity than the first layer so as to have a thermal conductivity which is at least 10% lower than a thermal conductivity of said first layer.

4. The process of claim 3, wherein said first layer forming step comprises suspending a powder feedstock in a liquid suspension and injecting said powder feedstock and said suspension into a plasma jet under conditions where said first layer is formed with said strain-tolerant columnar microstructure.

5. The process of claim 4, wherein said second layer forming step comprises changing spray parameters so as to form said porous and radiation thermally resistant second layer.

6. The process of claim 3, wherein said second layer forming step comprises forming said second layer so as to have a porosity of from 10 to 40%.

7. The process of claim 3, wherein said first and second layer forming steps comprise using a powdered feedstock having a particle size in the range of from 10nm to 10 micrometers.

8. The process of claim 7, wherein said first and second layer forming steps comprise using a powdered feedstock having a particle size in the range of from 10nm to 2 micrometers.

## Patentansprüche

1. Wärmedämmschicht (14), die auf eine Turbinenmotorkomponente (10) aufgebracht wird, die ein Substrat (2) aufweist, wobei die Schicht Folgendes umfasst:
eine erste Lage (16), die eine beanspruchungsfähige, säulenartige Mikrostruktur an einer Schnittstelle mit dem Substrat zur Beständigkeit gegenüber Zersplitterung aufweist; und
eine zweite Lage (20), die porös ist und beständig gegenüber Wärmeleitung und -strahlung, an einer Außenfläche der Wärmedämmschicht;
wobei eine kontinuierlich abgestufte Mikrostruktur von der Schnittstelle zur Außenfläche vorliegt;
wobei die erste und die zweite Lage aus demselben Material ausgebildet sind;
wobei jede aus der ersten und der zweiten Lage aus mit 7 Gew.-% Yttriumoxid dotiertem Zirkoniumdioxid ausgebildet ist; und wobei die erste Lage eine erste Wärmeleitfähigkeit aufweist und die zweite Lage eine zweite Wärmeleitfähigkeit aufweist, die um mindestens 10 % niedriger als die erste Wärmeleitfähigkeit ist.

2. Wärmedämmschicht nach Anspruch 1, wobei die zweite Lage eine Porosität im Bereich von 10 bis 40 % aufweist.

3. Verfahren zum Aufbringen einer Wärmedämmschicht (14) auf eine Turbinenmotorkomponente (10), umfassend:
Ausbilden einer ersten Lage (16), die eine beanspruchungsfähige, säulenartige Mikrostruktur aufweist, an einer Schnittstelle der ersten Lage und eines Substrats unter Verwendung einer Technik des Plasmaspritzens mit einer Suspension;
Ausbilden einer zweiten Lage (20), die porös ist und beständig gegenüber Wärmestrahlung, an einer Außenfläche der Wärmedämmschicht unter Verwendung der Technik des Plasmaspritzens mit einer Suspension;
Ausbilden einer kontinuierlich abgestuften Mikrostruktur von der Schnittstelle zur Außenfläche,
wobei die Schritte des Ausbildens der ersten und der zweiten Lage das Ausbilden dieser Lagen aus demselben Material umfasst;
wobei jede aus der ersten und der zweiten Lage aus mit 7 Gew.-% Yttriumoxid dotiertem Zirkoniumdioxid ausgebildet ist; und
wobei der Schritt des Ausbildens der zweiten Lage das Ausbilden der zweiten Lage mit einer höheren Porosität als die erste Lage umfasst, so dass sie eine Wärmeleitfähigkeit aufweist, die um mindestens 10 % niedriger als die Wärmeleitfähigkeit der ersten Lage ist.

4. Verfahren nach Anspruch 3, wobei der Schritt des Ausbildens der ersten Lage das Hängen eines Pulvereinsatzstoffes in eine flüssige Suspension und das Einspritzen des Pulvereinsatzstoffes und der Suspension in einen Plasmastrahl unter Bedingungen, unter denen die erste Lage mit der beanspruchungsfähigen, säulenartigen Mikrostruktur ausgebildet wird, umfasst.

5. Verfahren nach Anspruch 4, wobei der Schritt des Ausbildens der zweiten Lage das Ändern der Spritzparameter umfasst, so dass die poröse und wärmestrahlungsresistente zweite Lage ausgebildet wird.

6. Verfahren nach Anspruch 3, wobei der Schritt des Ausbildens der zweiten Lage das Ausbilden der zweiten Lage derart, so dass sie eine Porosität von 10 bis 40 % aufweist, umfasst.

7. Verfahren nach Anspruch 3, wobei die Schritte des Ausbildens der ersten und der zweiten Lage das Verwenden eines pulverisierten Einsatzstoffes mit einer Partikelgröße im Bereich von 10 nm bis 10 Mikrometer umfasst.

8. Verfahren nach Anspruch 7, wobei die Schritte des Ausbildens der ersten und der zweiten Lage das Verwenden eines pulverisierten Einsatzstoffes mit einer Partikelgröße im Bereich von 10 nm bis 2 Mikrometer umfasst.

## Revendications

1. Revêtement de barrière thermique (14) appliqué à un composant de moteur à turbine (10) ayant un substrat (2), ledit revêtement comprenant :
une première couche (16) qui a une microstructure en colonne tolérante à la contrainte au niveau d'une interface avec le substrat pour résistance à la spallation ; et
une seconde couche (20) qui est poreuse, thermiquement résistante au rayonnement et à la conduction au niveau d'une surface extérieure du revêtement de barrière thermique ;
dans lequel il y a une microstructure échelonnée en continu de l'interface vers la surface extérieure ;
dans lequel lesdites première et seconde couches sont formées à partir du même matériau ;
dans lequel chacune desdites première et seconde couches est formée à partir de 7 % en poids de zircone stabilisée par de l'oxyde d'yttrium ; et
dans lequel ladite première couche a une première conductibilité thermique et ladite seconde couche a une seconde conductibilité thermique qui est au moins 10 % inférieure à la première conductibilité thermique.

2. Revêtement de barrière thermique selon la revendication 1, dans lequel ladite seconde couche présente une porosité dans la plage de 10 à 40 %.

3. Procédé pour appliquer un revêtement de barrière thermique (14) à un composant de moteur à turbine (10) comprenant :
la formation d'une première couche (16) qui a une microstructure en colonne tolérante à la contrainte au niveau d'une interface de la première couche et d'un substrat en utilisation une technique de pulvérisation de plasma en suspension ;
la formation d'une seconde couche (20) qui est poreuse et thermiquement résistante au rayonnement au niveau d'une surface extérieure du revêtement de barrière thermique en utilisant ladite technique de pulvérisation de plasma en suspension ;
la formation d'une microstructure échelonnée en continu de ladite interface vers ladite surface extérieure ;
dans lequel lesdites étapes de formation de première et seconde couches comprennent la formation desdites couches à partir du même matériau ;
dans lequel chacune desdites première et seconde couches est formée à partir de 7 % en poids de zircone stabilisée par de l'oxyde d'yttrium ; et
dans lequel ladite étape de formation de seconde couche comprend la formation de ladite seconde couche avec plus de porosité que la première couche de manière à ce qu'elle ait une conductibilité thermique qui est au moins 10 % inférieure à une conductibilité thermique de ladite première couche.

4. Procédé selon la revendication 3, dans lequel ladite étape de formation de première couche comprend la suspension d'une charge de poudre dans une suspension liquide et l'injection de ladite charge de poudre et de ladite suspension dans un jet de plasma dans des conditions où ladite première couche est formée avec ladite microstructure en colonne tolérante à la contrainte.

5. Procédé selon la revendication 4, dans lequel ladite étape de formation de seconde couche comprend le changement de paramètres de pulvérisation de manière à former ladite seconde couche poreuse et thermiquement résistante au rayonnement.

6. Procédé selon la revendication 3, dans lequel ladite étape de formation de seconde couche comprend la formation de ladite seconde couche de manière à avoir une porosité de 10 à 40 %.

7. Procédé selon la revendication 3, dans lequel lesdites étapes de formation de première et seconde couches comprennent l'utilisation d'une charge de poudre ayant une taille de particule dans la plage de 10 nm à 10 micromètres.

8. Procédé selon la revendication 7, dans lequel lesdites étapes de formation de première et seconde couches comprennent l'utilisation d'une charge de poudre ayant une taille de particule dans la plage de 10 nm à 2 micromètres.
